

# United States Patent Office

2,764,529

Patented Sept. 25, 1956

1

2,764,529

## STEAM CYLINDER LUBRICATING OIL

Robert J. Leygonie, Notre-Dame, and Bernard B. de Saint Leger, Paris, France, assignors to Esso Standard Societe Anonyme Francaise, Paris, France, a body corporate

No Drawing. Application April 23, 1952,  
Serial No. 283,970

Claims priority, application France August 18, 1951

3 Claims. (Cl. 196—151)

This invention relates to steam cylinder lubricating oils and to a process for their preparation. Particularly the invention relates to mineral oils having high temperature and volatility characteristics which render them suitable for the lubrication of steam cylinders.

Steam cylinders in use in modern technology may be generally divided into three groups; saturated steam cylinders, operating at temperatures in the neighborhood of 300° to 320° C., moderately superheated steam cylinders which operate at 300° C. to 350° C., and highly superheated steam cylinders operating at temperatures in excess of 350° C.

Steam cylinder lubrication is ordinarily accomplished by introducing a lubricating oil with the steam (atomization) or by injecting the oil into the cylinder through small orifices in the cylinder, or by a combination of both techniques. It is to be seen, therefore, that steam cylinder lubricating oils are subjected to extremely severe conditions. They must possess heat stability characteristics such as to prevent their decomposition to tar or coke under prolonged high temperatures and to minimize tarry and sticky residues often deposited on the various lubricated parts. They must possess good low temperature properties in order to ensure circulation in the lubrication system at low temperatures. They must be sufficiently low in volatility to prevent entrainment and escape with steam during exhaust.

Cylinder oils are ordinarily highly refined mineral oils which may or may not contain incorporated therein various oxidized or non-oxidized fatty oils. The mineral oils used are mainly of three distinct types:

Type 1: Distillation residues of non-asphaltic, paraffinic crude petroleum (principally Pennsylvania petroleum), either treated or not with sulfuric acid.

Type 2: Very viscous distillates obtained under high vacuum, treated or not with sulfuric acid or selective solvents and, if necessary, dewaxed.

Type 3: The bright stocks or unfinished cylinder oils, obtained by propane deasphalting of distillation residues from asphalt-base crudes. These propane-extracted oils are generally refined by the usual means (sulfuric acid, selective solvents) and dewaxed.

The art has generally found that only type 1 oils, that is, those from the non-asphaltic paraffinic Pennsylvania crudes are suitable for the lubrication of highly superheated steam cylinders. Oils of type 2 or 3 are either rapidly entrained or give tarry or coke deposits on the lubricated parts. This is believed to be due to a lack of certain high molecular weight paraffinic fractions believed heretofore to be present only in the Pennsylvania type crudes.

It has now been found, and forms the object of this invention, that these certain high molecular weight paraffinic fractions, hereinafter referred to as resins, may be extracted from other crude sources other than the Pennsylvania crudes and combined with mineral oils to form steam cylinder oils which have outstanding high temperature characteristics.

2

Briefly stated the instant invention comprises treating an asphalt with a liquid mixture of butane and propane to extract the paraffinic and naphthenic components therefrom, treating the raffinate with a solvent that is selective for the naphthenic constituents and obtaining a highly paraffinic resinous material suitable for combining with highly refined mineral oils to prepare compositions suitable for the lubrication of steam cylinders.

The asphalt or asphaltic material which is used as a starting material may be any asphalt derived from crude petroleum, whether from vacuum distillation or from a propane deasphalting process. It is of especial note that asphalts obtained from such crudes as Venezuelan crudes or Arabian crudes are suitable starting materials.

The mixture of butane and propane may be varied between limits of about 10% propane to 30% propane preferably 15% to 20%, percentages being by volume. The propane tends to reduce the solvent power of the butane and tends to limit the solvating effect to those components of the asphalt that are desirable. To use more than about 30% of propane would reduce the solvent power of the mixture to the point where the heavier fractions would not dissolve and to use less than about 10% would increase the solvation effect of the mixture to a point where undesirable components would be extracted from the asphalt.

The amount of solvating mixture which is used to extract the asphalt base may be between about 5 volumes and 15 volumes, preferably 10 to 12 volumes, depending upon the component parts of the asphalt. The temperature of the treating step should be maintained at one within a range from —20° C. to 120° C., the preferred temperature range being about 70° C. to 100° C. Any of the commonly known methods of contacting, such as countercurrent towers, agitator-separator equipment and the like may be utilized in this extraction step.

The raffinate from the butane-propane extraction is then treated with a solvent that is selective for the naphthenic constituents. Although it is preferred to use anhydrous phenol it is also within the concept of this invention to use any of the naphthene selective solvents known in the art such as light hydrocarbons, ketones, chlorinated solvents and the like. If desired, a dewaxing solvent may also be incorporated into this naphthene extraction step.

The resulting resinous material containing high molecular weight paraffins and excluding any naphthenic constituents which are notably heat unstable, may be blended with various known highly refined mineral oils to obtain a steam cylinder lubricant. For example, one may use as a base stock a phenol-treated propane deasphalting Mid-Continent crude residuum and combine therewith from 10% to 40% by volume of the resinous material to obtain a highly successful steam cylinder oil. Percentages of the resinous material of from 15% to 35% by volume are especially preferred.

In order to test the composition of the instant invention a testing procedure was performed in a laboratory apparatus reproducing the conditions of temperature and pressure prevailing in steam cylinders. (Cf. Bancelin-S. N. C. F. method, Rev. Gen. Chim. de Fer. 11/1/37.) This testing procedure is as follows:

70 gr. of the test oil are poured into a calorimetric bomb which is placed along with a small superheater coil into an electric oven. Steam at 12 kg. pressure and superheated to the temperature of the test is bubbled through the oil for three hours, the oil being at the steam temperature. The entraining steam passes at a uniform rate such that after three hours three liters of liquid can be collected (condensed water plus entrained products).

## 3

Finally, the unentrained residue in the vessel is weighed. The oil passes the test at a given temperature, if at this temperature, the following observations are made:

- (1) At least 7 gr. of residue remains.
- (2) This residue is oily or greasy and does not contain hard matter (coke).

It is to be noted that steam cylinder oils of type 1 above pass this test easily at 400° C. Neither type 2 nor type 3 oils pass the test at 380° C.; type 2 failing at 350° C. A number of oils prepared according to instant invention have successfully passed this specifically designed test for steam cylinder lubricating oils. The preparation of these oils are set out in detail below.

## Example 1

10 volumes of commercial liquid butane (containing 15% by volume of liquid propane) were used to treat at 30° C. an asphalt having a penetration of 25 at 25° C. (A. S. T. M. D 5-25), obtained from the vacuum distillation in the presence of steam of mixed-base Venezuelan crude petroleum. A yield of 55% by weight of a green oil was obtained having the following characteristics.

Density at 15° C. 0.975  
Saybolt Universal viscosity at 210° F. 1113 } oil No. I

This oil was treated with 9.5 volumes of phenol in four stages under the following conditions:

1st treatment: 2 volumes of anhydrous phenol at 75° C.  
2nd treatment: 2 volumes of anhydrous phenol at 85° C.  
3rd treatment: 3 volumes of anhydrous phenol at 85° C.  
4th treatment: 2.5 volumes of anhydrous phenol at 90° C.

A raffinate was obtained in 40% yield having the following characteristics:

Density at 15° C. 0.924  
Saybolt Universal viscosity at 210° F. 567 } oil No. II

An oil of type 3 was prepared by deasphalting a Mid-Continent reduced crude with 10 volumes of propane at 45° C. The oil thus obtained was treated with phenol up to a viscosity index of 101. Its Saybolt Universal viscosity at 210° F. was 240. This oil is designated oil No. IV.

The following mixture was made:

Oil No. IV 70% by vol. } oil No. III  
Oil No. II 30% by vol. } oil No. IV

Oil No. IV gave, in the test mentioned above, a negative result at 385° C.

On the other hand, oil No. III gave, at 395° C., 10 gr. of an oily residue, and, at 400° C., 7 gr. of a residue having the appearance of a very thick brown-black oil.

## Example 2

An Arabian reduced crude having an Engler viscosity of 30° at 100° C. was deasphalting with propane at 45° C. and gave an asphalt having a penetration of 25 at 25° C. (A. S. T. M. D 5-25).

This asphalt was dissolved in 10 volumes of commercial liquid butane containing 15% propane.

The butane at 30° C. precipitated the asphaltenes and a viscous oil was separated from the butane layer. It is characterized as follows:

Density at 15° C. 0.999  
Saybolt Universal viscosity at 210° F. 1600 } oil No. V

Oil V was treated with anhydrous phenol under the following conditions:

1st treatment: 2.0 volumes of phenol at 75° C.  
2nd treatment: 2.5 volumes of phenol at 85° C.

A 25% yield of an oil was obtained having the following characteristics:

Density at 15° C. 0.946  
Saybolt Universal viscosity at 210° F. 868 } oil No. VI

## 4

This oil was mixed with oil No. IV in the following proportions:

Oil No. IV 70% by vol. } oil No. VII  
Oil No. VI 30% by vol. } oil No. VII

Cylinder oil No. VII thus obtained gave the following results in the test:

|            | Gram residue |
|------------|--------------|
| At 390° C. | 13           |
| At 400° C. | 6            |

In order to show the deleterious effect of the naphthenic constituents, removed by the phenol treating step, the following example is given:

15

## Example 3

The mixture

|            | Percent by volume |
|------------|-------------------|
| Oil No. I  | 30                |
| Oil No. IV | 70                |

20

when tested, gave at 390° C. 10 gr. of residue which was black and asphaltlike. At 395° C. only a carbonaceous residue was obtained.

It is readily seen from the foregoing examples that the materials prepared by the concept of instant invention are outstanding in their utility as steam cylinder lubricants. Materials prepared by the butane-propane extraction of asphalts followed by the removal of the naphthenic constituents from the raffinate by phenol treatment, contain the high molecular weight paraffinic resins which enable a type 3 oil to withstand stringent requirements existing in the high pressure steam cylinders.

To summarize briefly, this invention comprises the preparation of a steam cylinder lubricant by the steps of treating an asphalt with a mixture of butane and propane containing from 10% to 30% by volume of propane and treating the raffinate thus obtained with a solvent that is selective for the naphthenic constituents thereof. The resulting composition composed primarily of high molecular weight paraffinic materials may be blended with refined mineral oils to prepare steam cylinder lubricants having outstanding qualities of high temperature resistance, resistance to steam entrainment and viscosity characteristics. It is to be noted that in accordance with the instant invention the asphalt used as a starting material may not only be the straight run asphalts, that is, the residuum of asphalt base crude, but may also be the asphalts obtained by deasphalting oils such as those obtained by precipitation with propane or propane-phenol mixtures. It is, therefore, possible according to the instant invention to propane deasphalt a crude petroleum, treat the raffinate by subsequent refining techniques to obtain a refined mineral oil base stock, treat the asphalt by the process of this invention to obtain the resinous materials desired, and combine the two to greatly increase the yield of steam cylinder oils desirable.

What is claimed is:

1. A steam cylinder lubricating oil comprising a propane-deasphalting phenol treated Mid-Continent reduced crude containing combined therewith from 10% to 40% by volume of a high molecular weight paraffinic material obtained by treating an asphalt with from 10 to 12 volumes of a liquid mixture of butane and propane containing from 10% to 30% by volume of propane at a temperature within a range from 70° C. to 100° C. to obtain an extract containing both paraffinic and naphthenic components, extracting the extract thus obtained with anhydrous phenol, and obtaining therefrom said high molecular weight paraffinic material as a raffinate.
2. A steam cylinder lubricating oil comprising a highly refined mineral lubricating oil containing combined therewith from 10 to 40%, by volume of a high molecular weight paraffinic material obtained by treating an asphalt with a liquid mixture of butane and propane containing from 10 to 30% by volume of propane to obtain

an extract containing both paraffinic and naphthenic components, extracting the extract thus obtained with a solvent selective to the naphthenic components and obtaining therefrom said high molecular weight paraffinic material as the raffinate.

3. A steam cylinder lubricating oil comprising a propane-deasphalted reduced crude containing combined therewith from 15 to 35% by volume of a high molecular weight paraffinic material obtained by treating an asphalt with from about 5 to 15 volumes of a liquid mixture of butane and propane containing from 15 to 20% by volume of propane to obtain an extract containing both paraffinic and naphthenic components, extracting the extract thus obtained with a solvent selective to the naphthenic

components and obtaining therefrom said high molecular weight paraffinic material as the raffinate.

References Cited in the file of this patent

UNITED STATES PATENTS

|           |              |               |
|-----------|--------------|---------------|
| 1,988,712 | Bray et al.  | Jan. 22, 1935 |
| 2,081,496 | Merrill      | May 25, 1937  |
| 2,165,432 | Whiteley     | July 11, 1939 |
| 2,168,258 | Fisher       | Aug. 1, 1939  |
| 2,339,898 | White et al. | Jan. 25, 1944 |

FOREIGN PATENTS

|         |           |              |
|---------|-----------|--------------|
| 117,653 | Australia | Nov. 4, 1943 |
|---------|-----------|--------------|